

April 3, 1934.

J. C. BLACK ET AL

1,953,333

PROCESS FOR THE MANUFACTURE OF ASPHALTIC PRODUCTS

Filed Dec. 7, 1927



## UNITED STATES PATENT OFFICE

1,953,333

PROCESS FOR THE MANUFACTURE OF  
ASPHALTIC PRODUCTS

John C. Black, Los Angeles, and Wirt D. Rial,  
Watson, Calif., assignors, by mesne assignments,  
to Earle W. Gard, Palos Verdes Estates,  
Calif.

Application December 7, 1927, Serial No. 238,428

## 12 Claims. (Cl. 196—74)

This invention relates to a process for treating asphaltic residuum, and has particular reference to a method for producing a high grade asphalt suitable for any of the various uses in the art.

An object of the invention is to provide a simple, efficient and economical process by which asphaltic residuum may be converted into an asphaltic product, which will have a relatively high melting point and flash, and at the same time will be of a suitable ductility.

Another object of the invention is to provide a simple and efficient process for manufacturing asphaltic products, in which the various characteristics of ductility, high melting point and flash, required by different branches of the individual art, may be controlled, separately or combinedly. Another object of the invention is to provide a method by which asphaltic residuum may be uniformly oxidized to the required degree at a minimum consumption of time, and with a minimum consumption of the oxidizing agent.

Heretofore, difficulty has been experienced in providing an asphaltic material entirely suitable for the manufacture of roofing felt, battery sealing compounds, and the like, in which relatively high flash and high melting point materials are required, and one which will have suitable ductility at 77 degrees F. We have discovered that this is due to producing products which are not uniformly oxidized, in which some part of the asphaltic material has been overoxidized, while other parts have not been sufficiently oxidized to give the required melting point, flash and ductility.

We have discovered that these difficulties may be overcome by employing a smaller quantity of air and a longer time contact between the asphaltic oil and the air, in which case a partial oxidizing action is uniformly effected to the required degree in a much shorter time and without the formation of carbonaceous material.

In the conventional method of oxidizing asphaltic oils for the production of oxidized asphalt, air is introduced into a cylindrical still containing the asphaltic oil through a spray line and at the same time the asphaltic oil contained in the still is heated to a temperature sufficient to obtain the oxidizing reaction, approximately 450 to 550 degrees F. By such methods the air is only in contact with the asphaltic oil momentarily, passing upward through the depth of the oil in the still, thence out through the vapor line, carrying products of distillation, whereby excessive quantities of air must be employed to obtain the desired product. On account of the short time contact of the air with the asphaltic oil undergoing oxidation, a uniform oxidized product cannot be obtained, also a uniform temperature is difficult to maintain since the oxidizing reaction is exothermic and the added heat may overheat the as-

phaltic oil to a point of cracking or other decomposition reaction, thereby rendering the product more brittle or less ductile than it would be if a uniform oxidized product at a lower temperature could be made.

Also we have discovered that when excessive quantities of air, such as are employed in the conventional cylindrical batch still method, a higher percentage of distillation products is produced, which by our process are conserved and oxidized to desirable asphaltic products.

For example, by the conventional cylindrical batch still method the time required to convert a batch of asphaltic oil to an oxidized product suitable for the manufacture of roofing felt, requires approximately 24 hours or more, while by our invention the reaction is accomplished in about one half the time and the total quantity of air employed is approximately only 50 per cent of the air required by the conventional batch method.

In the manufacture of oxidized asphalt for coating roofing felt, or the like, by our invention we may obtain a product having the following tests:

|                      |                 |
|----------------------|-----------------|
| Penetration @ 77° F. | 15 to 18        |
| Melting point        | 225 to 260° F.  |
| Ductility            | 1.25 to 2.0 cm. |
| Flash                | 430 to 460° F.  |

We have found it advantageous to circulate a large amount of oil through the heating and air contact coil and a relatively small volume of air, the contact being over a prolonged period of time relative to the time of contact in a cylindrical still such as previously used in the art; by this procedure we are enabled to produce a superior finished asphaltic compound as the oxidation is not as severe with the result that less carbonaceous material is produced and greater ductility and penetration is obtained at a given flash and melting point.

We have also found that by maintaining a pressure on the heating and contact coil, oxidation may be hastened, or maintaining a definite rate of oxidation less air may be used; that is to say the air will be more effectively denuded of its oxygen content. This will represent a saving in compressed air as well as a saving in heat.

With the foregoing preliminary explanation the preferred embodiment of our invention will now be more fully explained by reference to the accompanying drawing, which is a diagrammatical representation of a preferred apparatus for carrying out the operations of the present invention.

In the drawing, Figure 1 represents the complete apparatus for carrying out the invention and Figure 2 shows the cross-section of the still 1 on "A"—"A".

65

70

75

80

85

90

95

100

105

110

115

120

In Figure 1, 1 represents generally a still or chamber for holding the bulk supply of oil, which may be externally heated. A pipe 2 connects the still 1 at the bottom to the inlet side of a steam jacketed pump 4 controlled by the valve 40. A pipe 8 controlled by the valve 3 is connected to the pipe 2 and leads to a source of asphaltic oil residuum not shown. A pipe 5, controlled by the valve 6 connects the discharge side of the pump 4 to pipe 32. A pipe 18 controlled by the valve 19 is connected to the pipe 32, and leads to a source of steam not shown. A pipe 21, controlled by valve 7 is connected to the pipe 32 and leads to a source of air not shown. The pipe 32 is connected to a heater coil 9 at the top. The heater and air contact coil 9 is interposed in the furnace 10 which is provided with a burner 11 which leads to a source of fuel not shown. A pipe 33 controlled by the valve 33' connects the heater coil 9 at the bottom to the still 1, passing through the shell of the still 1 near the top. A pipe 12 controlled by the valve 31 connects the pipe 5 to storage tank 13. A pipe 16 controlled by the valve 15 connects the steam pipe 14 to the still 1 near the top. The pipe 14 controlled by the valve 34 is connected to the spray line 17 which is in the still 1 near the bottom. A pipe 35 controlled by the valve 36, is connected to the steam pipe 14. The steam pipe 14 leads to a source of steam not shown. A vapor line 20 is connected to the still 1 at the top by the pipe fittings 27. The vapors may be taken to a condenser where the condensable materials are condensed by cooling fluid and the uncondensed vapors, gases and steam are withdrawn by means of a vacuum pump which will maintain the desired vacuum in the still 1. In Figure 2, which is a cross-section of the still 1 showing the connections of the vapor line 20 to the still 1, 42 is a cross fitting connected to the top of the still by means of a nipple 43. The pipe 26 connects the cross fitting 42 to the cross fitting 42'. The pipe 27 connects the cross fitting 42' to the vapor line 20 by means of a T. The pipes 33, 32, 2, 12 and 5 are preferably covered with a suitable insulating material to prevent any substantial loss of heat, or they may be steam jacketed.

The preferred process as carried out in the apparatus described is as follows:

50 Asphaltic oil, which may be any crude petroleum oil or preferably residuum derived by the distillation of an asphalt or mixed base crude petroleum oil, and preferably ranging in gravity from 10 or below to 16 degrees Bé., is charged into still 1 to a predetermined level by operating pump 4, which takes suction on the charging line 8 through the pipe 2. The charging line 8 leads to a source of supply not shown. During the charging of the still 1, valve 40 is closed and valve 3 is opened. The petroleum oil stock is discharged by the pump 4 into the pipe 5, valve 31 being closed and valve 6 being open. From pipe 5 the petroleum oil stock passes through the pipe 32, heater coil 9, pipe 33 and valve 33' and then into the still 1, valves 7 and 19 being closed. When still 1 contains a sufficient charge of the petroleum oil stock, valve 3 is closed and valve 40 is opened which permits the oil to circulate from the still 1 through the heating coil 9 and back to the still 1, or source of bulk supply. Heat is now applied to the furnace 10 by means of the burner 11 and regulated so that the oil passing through the heater coil 9 will attain a temperature of approximately 450 to 550 degrees F. or whatever temperature is desired for that particular run.

When the circulating oil has attained a suitable temperature and flash a regulated stream of air is introduced into the pipe 32 from the pipe 21, which leads to a source of compressed air not shown. In some cases it may be desired to introduce a small amount of air during the charging and heating of the oil.

The circulation of the oil at the oxidizing temperature and the introduction of the air are maintained for a period of time required to obtain the desired product, such time depending upon the quality of the oil employed, the product desired and the amount of air introduced. If desired, the oil and air passing through the heater coil 9 may be kept at any desired pressure above atmospheric, by regulating valve 33'. Also a vacuum may be maintained on the bulk supply chamber or still 1, whereby the oxidation is carried on at a still further reduced temperature.

In producing certain varieties of oxidized asphalt it may be found advantageous to introduce steam along with the air which is carried out by opening valve 19 sufficiently to admit the desired amount of steam from pipe 18 which decreases the time of reaction, and the tendency of the oil to crack, thereby producing a product of a superior quality.

During the oxidation of the asphalt with air or steam and air, the air, in conjunction with the products of distillation, passes from the still 1 into the vapor line 20. The vapor line 20 leads to a condenser not shown where the oil products are condensed and separated from the gases.

When the petroleum oil residuum has been oxidized to the required degree, it is discharged into the storage tank 13 passing from the bottom of the still 1 through the pipe 2, pump 4, pipe 5 and pipe 12, valve 31 being open and valve 6 being closed.

During the time that the still is being emptied of the finished oxidized asphalt, steam is admitted into the still 1 through the pipe 16 controlled by the valve 15. The pipe 16 is connected to the steam pipe 14 which leads to a source of steam not shown. The introduction of steam into the top of still 1 during the removal of the finished products of the still is carried out to prevent explosive mixtures from forming in the top of the still. Therefore the quantity of steam admitted into the still through the pipe 16 is just sufficient to fill the space above the liquid asphalt as it is being withdrawn.

In some cases where the oxidized asphalt is not at a sufficiently high flash after the oxidizing operation, the flash may be further raised by steaming the charge for a period of time. This is accomplished by the introduction of steam into the still 1 through the spray line 17 which is connected to the steam line 14 controlled by the valve 34. During this operation, in order to obtain a steam free from water, valve 36 is opened to a slight extent so as to permit any water to separate from the steam entering the spray line.

This reduction or steaming of the oxidized asphalt may also be accomplished by introducing steam into the circulating system from the steam pipe 18 by the proper regulation of valve 19 which is connected to the pipe 32 and leads to the heater coil 9 as heretofore described.

The operation of this invention for the production of an oxidized asphalt with a desired flash, melting point and ductility may be conducted various ways, for example, during the oxidation process both steam and air may be

admitted into the heating coil, or steam and air may be intermittently introduced into the heating coil. The regulation of each depends upon the stock under treatment and the product desired.

5 While the process herein described is well adapted for carrying out the objects of the present invention, it is to be understood that various modifications and changes may be made without departing from the spirit of the invention and the 10 invention includes all such modifications and changes as come within the scope of the appended claims.

What we claim is:

1. A process of forming oxidized asphalt comprising maintaining a bulk supply of asphaltic oil in a chamber at a pressure not greater than atmospheric and at a uniform oxidizing temperature, circulating the oil from the bulk supply to and through a heating coil and back to the bulk supply, introducing a regulated stream of air into the circulating oil, passing the oil commingled with air through the coil under a pressure greater than atmospheric and then separating the residual air with the products of distillation from the 25 oil.

2. A process of forming oxidized asphalt, comprising, maintaining a bulk supply of asphaltic oil in a chamber at a pressure substantially not greater than atmospheric, maintaining a substantially uniform, oxidizing temperature therein, by continuously circulating the oil from the bulk supply to and through a heating coil and back to the bulk supply, continuously introducing a regulated stream of air into the circulating oil before it enters the heating coil and continuously withdrawing the residual air and products of distillation from the chamber.

3. A process of producing asphalt which comprises passing a commingled stream of oil and air through a coil, maintaining said coil at an elevated temperature, maintaining superatmospheric pressure on said commingled oil and air in said coil, regulating the temperature and pressure and air to produce oxidized asphalt, and reducing the pressure on said oil and air and separating the asphalt from the vapors and gases under said reduced pressure.

4. A method of producing asphalt which comprises passing a commingled stream of oil and air through a coil, maintaining said oil in said coil at an elevated temperature, introducing said commingled stream of heated oil and air into a bulk supply chamber, separating the oxidized asphalt from the gases in said bulk supply chamber under vacuum.

5. A process of producing asphalt which comprises passing a commingled stream of oil and air through a coil, maintaining said coil at an elevated temperature, but insufficient to substantially crack said oil, maintaining superatmospheric pressure on said commingled oil and air in said coil, regulating the temperature and pressure and air to produce oxidized asphalt, and reducing the pressure on said oil and air and separating the asphalt from the vapors and gases under said reduced pressure.

6. A method of producing asphalt which comprises passing a commingled stream of oil and air through a coil under superatmospheric pressure, maintaining said coil in said coil at an elevated temperature, introducing said commingled stream of heated oil and air into a chamber maintaining said chamber under vacuum, separating

the oxidized asphalt from the gases under vacuum.

7. A method of producing asphalt which comprises passing a commingled stream of oil and air through a coil, maintaining said oil in said coil at an elevated temperature, but insufficient to substantially crack said oil, introducing said commingled stream of heated oil and air into a chamber maintaining said chamber under vacuum, separating the oxidized asphalt from the gases under vacuum.

8. A method of producing asphalt which comprises passing a commingled stream of oil and air through a coil under superatmospheric pressure, maintaining said oil in said coil at an elevated temperature, but insufficient to substantially crack said oil, introducing said commingled stream of heated oil and air into a chamber maintaining said chamber under vacuum, separating the oxidized asphalt from the gases under vacuum.

9. A method of producing asphalt which comprises maintaining a bulk supply of oil, circulating oil from said bulk supply introducing air into the circulating oil through a coil, maintaining said oil in said coil at an elevated temperature, introducing said commingled stream of oil and air into said bulk supply chamber, maintaining said chamber under vacuum, separating the gases and oil from the vapors under vacuum in said chamber, removing the oil and gases from said chamber and removing the asphalt from said chamber.

10. A method of producing asphalt which comprises maintaining a bulk supply of oil, circulating oil from said bulk supply introducing air into the circulating oil through a coil under superatmospheric pressure, maintaining said oil in said coil at an elevated temperature, introducing said commingled stream of oil and air into said bulk supply chamber, maintaining said chamber under vacuum, separating the gases and oil from the vapors under vacuum in said chamber, removing the oil and gases from said chamber and removing the asphalt from said chamber.

11. A method of producing asphalt which comprises maintaining a bulk supply of oil, circulating oil from said bulk supply introducing air into the circulating oil through a coil, maintaining said oil in said coil at an elevated temperature, but insufficient to substantially crack said oil, introducing said commingled stream of oil and air into said bulk supply chamber, maintaining said chamber under vacuum, separating the gases and oil from the vapors under vacuum in said chamber, removing the oil and gases from said chamber and removing the asphalt from said chamber.

12. A method of producing asphalt which comprises maintaining a bulk supply of oil, circulating oil from said bulk supply introducing air into the circulating oil through a coil under superatmospheric pressure, maintaining said oil in said coil at an elevated temperature, but insufficient to substantially crack said oil, introducing said commingled stream of oil and air into said bulk supply chamber, maintaining said chamber under vacuum, separating the gases and oil from the vapors under vacuum in said chamber, removing the oil and gases from said chamber and removing the asphalt from said chamber.

JOHN C. BLACK.  
WIRT D. RIAL.